

# UNITED STATES PATENT OFFICE.

HENRI PABAN, OF MARSEILLE, FRANCE, ASSIGNOR TO HIMSELF AND ALEXIS GRAWITZ,  
OF MARSEILLE, FRANCE.

## ILLUMINATED AIMING APPARATUS OR THE LIKE.

1,304,702.

Specification of Letters Patent. Patented May 27, 1919.

No Drawing.

Application filed January 4, 1919. Serial No. 269,721.

*To all whom it may concern:*

Be it known that I, HENRI PABAN, citizen of the Republic of France, and resident of Marseille, France (post-office address 25 Rue 5 de la Darse), have invented a new and useful Illuminated Aiming Apparatus or the like, which improvements are fully set forth in the following specification.

This invention relates to illuminated aiming apparatus or the like, and its comprises an improved process whereby the figures, graduations and other markings provided on apparatus of the character indicated as well as on other apparatus of like nature, are 10 rendered legible at night and, similarly, at other times and under other conditions where they would ordinarily be difficult if not impossible to read.

It was originally attempted to utilize electric lighting devices for the purpose indicated, but those devices were found to be thoroughly unsatisfactory owing to the liability of the lamps and their wires to be broken, cut or otherwise injured during the 20 course of an attack, and at other times when frequent firing occurs. Consequently, such lighting systems were ultimately discarded, and the markings were outlined directly upon the sights or analogous parts of the apparatus and in some suitable radio-active material which was usually applied upon thin strips of foil which, in turn, were covered with a layer or coating of mica or other transparent material.

30 In adopting that method, however, the difficulty of constructing and applying the illuminated markings proved so great that only dots or points and straight strokes could be utilized, which were insufficient to 35 accomplish the required purpose.

The present invention has for its object a method or process whereby the markings, irrespective of their character, are given a degree of luminosity which enables them to 45 be easily read in the dark and which is increased by the contrasting background whereon they appear.

According to the form of the invention which is now deemed preferable, the markings are etched, engraved or otherwise cut at the proper points in the surface of the copper or other metal of which the sight or analogous part of the apparatus or device is

constructed, and this cut or engraved surface is then covered or coated with a thin 55 film or layer of insulating material to prevent the subsequently-applied radio-active substance from coming into contact with the metal and being injuriously affected thereby. Silver has proven most satisfactory for this 60 purpose, and it may be applied in any desired manner, preferably by being deposited electrolytically upon the metal, and since it is interposed between the radio-active substance and the metal surface, it will prevent 65 any chemical reaction between the two which might tend to dim or otherwise impair the luminosity of the radio-active salt or salts with which, as will be understood, the markings are picked out or outlined after the 70 coating of silver or other material has been deposited upon the metal. The whiteness of the silver, however, precludes it from offering any vivid contrast to the luminous markings, particularly in daylight, when the 75 markings themselves have a whity appearance; and to overcome this objection, the layer of silver is treated chemically, or in some other manner, with a substance or material which will tarnish or darken it, so that 80 it will then form a dark or contrasting background on which the luminescent markings will stand out sharply. One way in which this object may be accomplished, is to subject the coated surface to a sulfureting action 85 by placing the sight or other part in a closed receptacle through which a current of sulfured hydrogen is passed, the operation being facilitated by slightly heating the receptacle. Other methods of sulfuration 90 may, of course, be substituted for the one just mentioned, as the invention resides in the step itself in its relation to the preceding steps, rather than in the particular manner in which it is carried out; but the method 95 described may be considered for all present purposes as preferred, the action of the sulfur imparting a grayish tint to the silver which shades rapidly into black.

In case the sights or equivalent parts are 100 constructed of a metal other than copper,—iron for example,—or if they are constructed of a non-metallic substance or material, the surface on which the markings are to be made will first be coated with copper in 105 some suitable way and thereafter treated in

the manner above described, the copperized surface having the markings subsequently engraved or etched upon it.

What is claimed, is:

- 5 1. The herein-described process, which consists in applying a coating of insulating material upon a metallic surface having markings engraved or cut thereon; outlining the markings with a radio-active material upon the insulating coating, whereby the radio-active material is prevented from contacting with the metal surface; and darkening the said coating, so as to form a background against which the markings stand out sharply.
- 10 2. The herein-described process, which consists in applying a coating of insulating material upon a metallic surface; marking outlines in luminous salts upon said coated surface, whereby said salts are prevented from contacting with the copper; and darkening the coating so as to form a background against which the markings stand out sharply.
- 15 3. The herein-described process, which consists in applying a coating of silver upon a metallic surface; marking outlines in luminous material upon the silver-coated surface, whereby the luminous material is prevented from contacting with the copper; and darkening the coating so as to form a background against which the markings stand out sharply.
- 20 4. The herein-described process, which consists in applying a coating of silver upon a metallic surface; marking outlines in luminous material upon the silver-coated sur-

face, whereby the luminous material is prevented from contacting with the metallic surface; and subjecting the said coating to a sulfureting action to darken it and thereby form a background against which the markings stand out sharply.

5. The herein-described process, which consists in applying a bright metallic coating upon a metallic surface having markings engraved thereon; outlining the markings in luminous material upon the metal coating, whereby the luminous material is prevented from contacting with the metal surface upon which said coating is applied; and darkening the said coating so as to form a background against which the margins stand out sharply.

6. The herein-described process, which consists in applying a bright metallic coating upon a metallic surface having markings engraved thereon; outlining the markings in luminous material upon the metal coating, whereby the luminous material is prevented from contacting with the metal surface upon which said coating is applied; and subjecting the said coating to a sulfureting action, so as to darken it and thereby form a background against which the markings stand out sharply.

In testimony whereof I have signed this specification in the presence of two subscribing witnesses.

HENRI PABAN.

Witnesses:

ALPHONSE KONIG,  
JOHN TRACEY.

Copies of this patent may be obtained for five cents each, by addressing the "Commissioner of Patents, Washington, D. C."